

## UNITED STATES PATENT OFFICE.

GEORGE A. WALKLEY, OF WESTFIELD, MASSACHUSETTS.

## LIGHT-WEIGHT AGGREGATE.

No Drawing.

Application filed January 23, 1920. Serial No. 353,638.

*To all whom it may concern:*

Be it known that I, GEORGE A. WALKLEY, a citizen of the United States of America, residing at Westfield, in the county of 5  
5 Hampden and State of Massachusetts, have invented certain new and useful Improvements in Light-Weight Aggregates, of which the following is a specification.

This invention relates to a process for 10 making a light weight aggregate suitable for construction purposes. While the process is independent of the use to which the product is put, it may be pointed out that the product is particularly advantageous as 15 an aggregate in the making of concrete.

Broadly considered, the invention consists in making a plastic mixture of a suitable brick-forming material, such as clay, with a combustible material, such as coal dust, saw dust or the like, and subsequently burning the mixture in a manner similar to brick burning, but more rapidly and with sufficient heat to harden the material into a strong compact form of porous density, but 20 not with high enough heat to draw the material together into a vitrified solid mass.

In a general way, the invention is carried out as follows; the clay and combustible material are thoroughly ground together 25 with water until the mass is of the desired plasticity, in a manner analogous to that employed in the art of brick making, as in a pug mill. The plastic mass is then preferably molded into blocks which are partially dried to a degree sufficient to permit stacking; the blocks are then stacked into a kiln and the latter fired; characterized in that the fire is forced rapidly to supply an intense heat and maintained continuously so 30 that the emission of the water-smoke is uninterrupted.

The process is characterized by its relative rapidity over the usual methods of burning brick. The usual complete drying 35 of the bricks in the present process is, in practical effect, omitted as only partial drying of relatively short duration is employed and for the purpose specified. The actual

burning process is also comparatively rapid, the fire being rushed from the start to the 50 end of this step of the process.

Other features of the invention will appear in the following more detailed description.

The preliminary step of the process consists in the thorough mixture of the materials to be burned. Broadly, the major element of this mixture is a suitable clay, and various clays may be used. It has been found that a particular kind of clay, technically known as soft shale, is especially adapted for this process, but the process is not confined to the use of this specific kind of clay although it is at present preferred.

For the combustible element of the mixture, various materials may be employed, but coal is particularly suitable, when in finely subdivided form, as it readily lends itself to admixture with the clay and may be distributed therethrough with substantial 65 uniformity. Preferably, coal dust, either of anthracite or bituminous coal, may be used although a mixture of anthracite with a long flame bituminous coal has proved in practice particularly satisfactory.

The proportions of the clay and combustible elements may be varied within wide limits, as desired, to effect varying degrees of porosity and thus control the density of the product. Exact proportions of the two 70 main ingredients are, therefore, not essential to success in practicing the process. In actual practice, these two ingredients are seldom measured with any degree of accuracy, but it may be stated that, with the particular combustible and the particular kind of clay mentioned, a suitable light weight aggregate is obtained by a mixture of nine parts of clay to one part of coal dust.

Preferably, although not necessarily, 75 there is added to the main elements described a suitable flux, such as a mixture of sulphur and borax for example. Generally, this is applied as a sprinkling to each batch as it is made up. For example, a batch 80 weighing approximately 2000 pounds will

consist of about 1800 pounds of clay, 200 pounds of coal dust and a handful of sulphur and a handful of borax.

The mixing of the constituents described 5 may be accomplished in any suitable manner. They may, however, be mixed to advantage in a manner analogous to that employed in the art of brick making, as by placing the constituents in a pug mill which 10 operates to thoroughly grind and mix the materials. At this time, water is added to the mixture until it is rendered of sufficient plasticity. These steps are substantially like those usually employed in brick making.

15 The mass, having been brought to the desired degree of plasticity, is then preferably molded into blocks or bricks, preliminary to the step of burning. The purpose of this step is merely to facilitate burning. That 20 is, the question of the final size and shape of the burned product is not ordinarily of particular importance, but it is convenient to mold the mass into bricks so that they can readily be stacked into kiln form for the 25 step of burning.

Before the bricks are burned, they are partially dried, as distinguished from complete drying customary in the preparation of ordinary bricks for burning in a kiln. 30 The purpose of this step is merely to dry the bricks to a degree sufficient to permit them to be stacked into a kiln.

The burning of the kiln is generally analogous to the burning of a kiln of ordinary 35 bricks with the exception that the firing throughout is more rapid than in ordinary brick burning. The fuel may be chosen as desired except that a fuel which will quickly yield an intense heat and lend itself to 40 forcing is preferable. Contrasted with ordinary brick burning, the fire is forced throughout to a relatively intense heat, and followed up to prevent diminution of the heat. The purpose of firing in this manner 45 is to quickly cause the generation of gases in the plastic bricks and to continue the generation and emission of gases from the bricks without interruption until exhaustion of the sources of gas. The degree of heat 50 employed is gauged to effect the results just named. Generally, the bricks are heated from 1700° to 1900° Fahr. The gases, which are commonly termed "water-smoke", are forced from the bricks in a continuous 55 manner by forcing the fires for this purpose. The characteristic feature of the step of burning is the rapid and intense initial heat and the forcing and "following up" 60 of the fire to secure complete emission of the gases. The time of rapid and intense firing is gauged by watching the emission of the water-smoke. For example, at the start of the step of burning the operator forces his fire to higher and higher temperatures until 65 he observes the emission of the water-smoke.

He then continues forcing the fire and never allows it to slacken until he is assured from the cessation of water-smoke, even under intense heat, that the exhaustion of the sources of gas is complete. After the emission of 70 water-smoke has ceased, the burning may be continued for a short time, if desired, but care should be taken not to burn the bricks into a vitrified solid mass. A higher degree 75 of heat than 2000° Fahr. or a continued heating after the water-smoke has been expelled from the brick will generally cause vitrification of the brick into a solid dense mass which it is desired to avoid in this process.

80 By carrying out the present process as described, it will be found that the brick is burned to a strong tough body of porous density so as to be extremely light as compared to ordinary brick. The bricks formed by the present process will generally be found to be swelled to a larger size than the original molded blocks and with rounded or bulging sides. In other words, they have the appearance of being blown up like 85 raised and baked bread.

90 The bricks when thus finished may be used as ordinary bricks, but may also be broken up into pieces of the desired size to 95 serve as an aggregate of concrete. The advantages of a strong light weight aggregate for such purpose is apparent.

What I claim is—

1. The process of making a light weight aggregate, which consists in mixing clay and finely divided fuel into a plastic mass, forming the mass into separate units, partially drying such units sufficiently for stacking into a kiln, stacking the units into a kiln, and in then rapidly firing the kiln 100 with an intense heat.

105 2. The process of making a light weight aggregate which consists in mixing clay and finely divided fuel into a plastic mass, forming the mass into separate units, partially drying such units sufficiently for stacking into a kiln, stacking the units into a kiln, and in then rapidly firing the kiln to a 110 temperature approximately between 1700° Fahr. and 1900° Fahr.

115 3. The process of making a light weight aggregate, which consists in mixing clay and finely divided fuel into a plastic mass, forming the mass into separate units, partially drying such units sufficiently for stacking into a kiln, stacking the units into a kiln, in then rapidly firing the kiln to a 120 temperature approximately between 1700° Fahr. and 1900° Fahr., and continuing said firing of the kiln until all apparent water-smoke has been driven off.

125 4. The process of making light weight aggregate, which consists in mixing clay and finely divided coal into a plastic mass in approximate proportions of nine parts 130

of clay and one part of coal and subjecting the same to a temperature of approximately between 1700° and 1900° Fahr. for a sufficient length of time to harden the same into a porous, burned clay product, but not sufficient to vitrify the same into a solid non-porous structure.

5. The process of making light weight aggregate, which consists in mixing clay and finely divided coal into a plastic mass

in approximate proportions of nine parts of clay and one part of coal, together with traces of sulphur and borax added as a flux, and subjecting the same to a temperature of approximately between 1700° and 1900° Fahr. for a sufficient length of time to harden the same into a porous, burned clay product, but not sufficient to vitrify the same into a solid non-porous structure.

10 GEORGE A. WALKLEY.